# EUROPEAN PATENT SPECIFICATION

(11) **EP 4 281 613 B1**
(45) Date of publication and mention of the grant of the patent: **13.05.2026**
(21) Application number: 22742951.1
(22) Date of filing: 19.01.2022
(51) Int. Cl.: D21F 11/02, D21F 1/48, D21F 9/02, D21H 21/56, D21F 11/00

(54) **METHOD FOR PRODUCING 3D FIBER STRUCTURES**
VERFAHREN ZUR HERSTELLUNG VON 3D-FASERSTRUKTUREN
PROCÉDÉ DE PRODUCTION DE STRUCTURES DE FIBRES 3D

(30) Priority: 19.01.2021 SE 2150053
(43) Date of publication of application: 29.11.2023
(73) Proprietor: Fibu AB, 734 32 Hallstahammar (SE)
(72) Inventor: ALIMADADI, Majid, 725 97 Västerås (SE)
(74) Representative: Zacco Sweden AB
(86) International application number: PCT/SE2022/050055
(87) International publication number: WO 2022/159019

(56) References cited:
- WO-A1-88/05096
- WO-A1-88/05096
- WO-A1-93/00471
- WO-A1-93/00471
- US-A- 3 542 640
- US-A- 3 542 640
- US-A- 3 716 449
- US-A- 3 716 449
- US-A1- 2020 190 739

## Description

### TECHNICAL FIELD

The present disclosure relates to a method for producing 3D fiber structures.

### BACKGROUND ART

Fiber network is an abundant structure among biological (e.g., animal tissues) and industrial materials which its characteristics is determined by individual elements' properties, orientation distribution, local and bulk density, bonding and entanglement between network elements. The morphology of many of biological fibrous structures are three-dimensional (3D) while manmade structures like paper and nonwoven are considered as two-dimensional (2D). In 3D fibrous structures, the constituent fibers are randomly oriented in the 3D space and the material bulk properties are distributed relatively uniform in all directions. In a 2D fibrous structure where constituent fibers are randomly oriented in the *plane* of the structure, in-plane bulk properties are drastically different compared to that of the normal direction to the plane. Unlike conventional paper, a 3D wood fiber structure is bulky, highly porous, and soft. These properties makes the 3D wood fiber structure a suitable candidate for applications related to absorption properties (shock, noise, moisture) and material transport properties (filtration).

Industrial fibrous structures are made from synthesized or natural fibers using dry- or wet-laying processes where in the latter process, water is used as the carrier medium for the fibers. Alternatively, aqueous foam can be used as the suspending phase to obtain a 3D fiber network which with existing methods the procedure is energy-intensive and time-consuming and therefore it is industrially unfavorable.

US3716449 A discloses forming of non-woven fibrous webs and in particular to the production of such webs utilizing a liquid suspending medium in the form of an aqueous foam in which the fibers are dispersed and suspended and from which they are formed into a layer on the wire of a paper-making machine, which layer is then collapsed and drained to form the web.

US3542640 A discloses a method for drying a wet foam containing randomly dispersed fibers by drying the wet foam in a series of steps to produce low density, absorbent, fibrous paper or sponge-like material. The foam is deposited is deposited as a uniform sheet on a moving foraminous support where most of the water is removed by drainage. The remaining water in the foam is removed by phase change. Water removal by phase change may include one or the other or both of the steps of impinging a hot gas normal to at least one surface of the wet sheet and/or blowing a hot gas through the sheet.

WO8805096 A1 discloses a method for the manufacture of very low density mineral wool structural panels on a moving foraminous support wire. A dilute aqueous furnish of mineral wool, lightweight aggregate, cooked wheat starch, cationic guar gum and non-ionic surfactant is formed, mixed to form a small amount of delicate non-resilient bubbles and ionically couple the mineral surfaces to the starch and gum, and deposited upon the wire to form an open, porous entangled mass which is rapidly stripped of water and dried in a flow-through configuration .

Accordingly, there is a need for an improved method which satisfies the accelerated dewatering of the excess water from a foam-formed fibrous mat without deteriorating the bulk of the structure.

### SUMMARY

It is therefore an object of the present disclosure to provide a method for producing 3D fiber structure to mitigate, alleviate or eliminate one or more of the above-identified deficiencies and disadvantages.

This object is achieved by means of a method as defined in the appended claims.

In accordance with the invention there is provided a method according to claim 1.

The present disclosure relates to a method for producing 3D fiber structures, preferably 3D wood fiber structures, the method comprising the steps of: Firstly, feeding a foamed fiber furnish to an apparatus, the apparatus comprising a liquid-permeable substrate means having a first side and an opposing second side, a dispenser having an outlet, wherein at least one of the dispenser and the substrate means travel with respect to the other. Further the method comprises the steps of: Dispensing, by means of the dispenser, a layer of foamed fiber furnish (or foamed wood fiber furnish) to the first side of said liquid-permeable substrate means to obtain a fibrous mat, wherein the apparatus further comprises at least a reservoir to facilitate an initial natural dewatering of the said fibrous mat for a predetermined time period, and a first vacuum unit associated with the second side of the liquid-permeable substrate means so to collect fluid discharge from the said fibrous mat. The method further comprises the step of applying at least a first dewatering pressure to at least a part of the second side of said substrate means. It should be noted that the foamed fiber furnish applied to the substrate means, takes the form of a fibrous mat. Thus, a layer of foamed fiber furnish is equal to a fibrous mat.

The layer of foamed fiber furnish is dispensed so to comprise a predefined substantially uniform thickness, wherein the apparatus is configured to, preceding the step of applying a dewatering pressure (which may also referred to as suction), by means of the reservoir, collect fluid discharge for a first period of time based on at least the thickness of the layer. The first period of time is in the range of 1-10 minutes The thickness of the layer is in the range of 1-10 cm.

The first dewatering pressure is applied for a second period of time, wherein the first dewatering pressure is within the range of 70 kPa - 100 kPa (i.e. slightly below atmospheric pressure providing a low suction). The second period of time is in the range of 2-10 minutes, preferably for 4-6 minutes.

A benefit of the method is that it allows for effectively producing a 3D fiber structure by maintaining an initial connected fiber network after a first natural dewatering which facilitates the use of vacuum pressure to more effectively discharge excess water without deteriorating the bulk of the said fibrous mat. Further, the method allows for a reduced drying time of the fibrous mat to up to 30% compared to solutions not involving vacuum pressure.

Further, in aspects, the liquid-permeable substrate means travels in a first direction along a traveling element having a length defined by at least a first and a second portion, wherein the dispenser is arranged to be above the first side of the substrate means in said first portion, wherein the reservoir is arranged in said first portion, wherein the first vacuum unit and a second vacuum unit are arranged sequentially along the length in said second portion, wherein the first vacuum unit is closer to the reservoir than the second vacuum unit. A benefit of this is that it allows for an arrangement where the fibrous mat is produced in a continuous process instead of a batch-wise process.

Thus, reservoir may collect some liquid, wherein the remaining of the water/liquid discharge may be carried out at the vacuum boxes and fibrous mat can then travel forward to a subsequent process.

The dispenser may be a headbox. Further the outlet may be a nozzle configured to dispense the fiber furnish with a defined shear force.

The first vacuum unit may be configured to apply a first dewatering pressure, wherein the second vacuum unit may be configured to apply a second dewatering pressure (thus applying a first and a second suction), wherein the first dewatering pressure is greater than the second dewatering pressure. The first vacuum unit may apply a first dewatering pressure being slightly below atmospheric pressure and wherein the second vacuum unit may apply a second dewatering pressure at a higher vacuum. The second dewatering pressure may be within a range of 50 kPa - 80 kPa. In some embodiments, the first and the second dewatering pressure are the same.

The method may further comprise the step of, simultaneous or preceding the step of applying the first dewatering pressure by applying an ultrasonic radiation to the said fibrous mat. The ultrasonic radiation may be performed by a high power airborne ultrasonic unit.

A benefit of this is that the ultrasonic energy facilitates a uniform collapse of foam bubbles throughout the thickness of the said fibrous mat without deteriorating the bulk of the structure while it also makes the fibrous mat highly permeable to air. Consequently, a faster discharge of excess water is possible and as a result the vacuum units may be arranged closer to the dispenser which makes it possible to use the space more efficiently. Additionally, an air permeable fibrous mat facilitates the utilization of more efficient drying technique, i.e., through air drying technology.

The substrate means may travel in the first direction with a velocity in the range of 0.1 - 10 m/s.

The method may further comprise the step of storing the dewatered fibrous mat at a temperature in the range of 70-120 °C.

The foamed fiber furnish comprises a fiber consistency in the range of 0.5-10% based on a dry weight of the fibers, wherein the foamed fiber furnish comprises a total concentration of foaming agents in the range of 0.05-2 g/l, wherein the foamed fiber furnish comprises an air content in the range of 55-70% by volume, wherein the foamed fiber furnish is generated from a pulp slurry. The thickness of dried fibrous mat may be in the range of 5 mm - 60 mm. Thus, the thickness of the mat provided by the method in accordance with the present disclosure may be 5 mm - 60 mm and is a 3D fiber structure.

There is further described an apparatus for producing 3D fiber structures, the apparatus comprising: a liquid-permeable substrate means having a first side and an opposing second side, a dispenser having an outlet, wherein at least one of the dispenser and the substrate means travel with respect to the other, a reservoir, at least a first vacuum unit, wherein the apparatus is configured to perform the method in accordance with the present disclosure. The apparatus may further comprise a second vacuum unit and an ultrasonic unit.

### BRIEF DESCRIPTION OF THE DRAWINGS

In the following the invention will be described in a non-limiting way and in more detail with reference to exemplary embodiments illustrated in the enclosed drawings, in which:
- Figure 1: illustrates from a side-view an apparatus in accordance with an embodiment of the present disclosure;
- Figure 2: illustrates from a side-view an apparatus in accordance with an embodiment of the present disclosure, the apparatus having a reservoir and a first and a second vacuum unit;
- Figure 3: illustrates an apparatus in accordance with an embodiment of the present disclosure, the apparatus having a reservoir, a first and a second vacuum unit and an airborne ultrasonic unit;
- Figure 4: illustrates the apparatus of Figure 1 having a layer of foamed fiber furnish on the substrate means;
- Figure 5: illustrates a method for producing 3D fiber structure in accordance with an embodiment of the present invention;
- Figure 6: illustrates a method for producing 3D fiber structure in accordance with an embodiment of the present invention;
- Figure 7A: illustrates a representation of a single fiber orientation in a 2D fibrous structure;
- Figure 7B: illustrates a representation of a single fiber orientation in a 3D fibrous structure.

### DETAILED DESCRIPTION

In the following detailed description, some embodiments of the present disclosure will be described. However, it is to be understood that features of the different embodiments are exchangeable between the embodiments and may be combined in different ways, unless anything else is specifically indicated. Even though in the following description, numerous specific details are set forth to provide a more thorough understanding of the provided method and apparatus, it will be apparent to one skilled in the art that the method and apparatus may be realized without these details. In other instances, well known constructions or functions are not described in detail, so as not to obscure the present disclosure.

Figure 1 illustrates an apparatus 1 for producing 3D fiber structures. The apparatus 1 comprises a liquid-permeable substrate means 3 having a first side 4 and an opposing second side 5, a dispenser 6 having an outlet 7, wherein at least one of the dispenser 6 and the substrate means 3 travel with respect to the other. In some embodiments the dispenser 6 is arranged to have a fixed position so that the substrate means 3 travels relative the dispenser 6 in a first direction x1.

The apparatus 1 shown in Figure 1 further comprises at least a reservoir 8 and a first vacuum unit 9 associated with the second side 5 of the liquid-permeable substrate means 3 so to collect fluid discharge from the dispensed layer 2 of foamed fiber furnish. As seen in Figure 1 the reservoir 8 and the first vacuum unit 9 may be integrated.

Figure 2 shows the apparatus 1 wherein the apparatus 1 also comprises a second vacuum unit 9'.

Figure 3 shows the apparatus 1 wherein the apparatus 1 also comprises an ultrasonic unit 12.

Figure 4 shows the apparatus 1 in Figure 1 wherein there is a layer 2 of foamed fiber furnish applied on the substrate means 3 traveling in a first direction x1.

Figure 5 schematically illustrates a method 100 for producing 3D fiber structures, the method 100 comprising the steps of: feeding 101 a foamed fiber furnish 2 to an apparatus 1 e.g. any of the apparatus 1 shown in Figures 1-3, the apparatus 1 comprising a liquid-permeable substrate means 3 having a first side 4 and an opposing second side 5, a dispenser 6 having an outlet 7, wherein at least one of the dispenser 6 and the substrate means 3 travel with respect to the other. Further comprising the step of dispensing 102, by means of the dispenser 6, a layer 2 of foamed fiber furnish to the first side of said liquid-permeable substrate means 3, wherein the apparatus 1 further comprises at least a reservoir 8 and a first vacuum unit 9 associated with the second side 5 of the liquid-permeable substrate means 3 so to collect fluid discharge from the dispensed layer 2 of foamed fiber furnish. Further comprising the step of applying 103 at least a first dewatering pressure to at least a part of the second side 5 of said substrate means 3. The first dewatering pressure may be applied for a second period of time, wherein the first dewatering pressure is within the range of 70 kPa - 100 kPa.

The layer 2 of foamed fiber furnish may be dispensed so to comprise a predefined substantially uniform thickness, wherein the apparatus 1 may be configured to (as seen in Figure 5), preceding the step of applying a first dewatering pressure 103, by means of the reservoir 8, collect 104 fluid discharge for a first period of time based on at least the thickness of the layer 2. The first period of time may be 1-10 minutes, wherein the second period of time may be 2-10 minutes, wherein the thickness of the layer 2 is within the range of 1-10 cm.

As shown in the apparatus in Figures 2 and 3, the liquid-permeable substrate means 3 may travel in a first direction x1 along a traveling element 13 having a length L1 defined by at least a first and a second portion 15', 15", wherein the dispenser is arranged to be above the first side of the substrate means 3 in said first portion 15', wherein the reservoir 8 is arranged in said first portion 15', wherein the first vacuum unit and a second vacuum unit 9, 9' are arranged sequentially along the length L1 in said second portion 9', wherein the first vacuum unit 9 is closer to the reservoir 8 than the second vacuum unit 9'. The traveling element 13 may be any suitable traveling element 13 that allows the substrate means 3 to travel along a length L1. Accordingly, the length L1 may also be defined as the working length (i.e. the distance between two points where the apparatus performs the steps in the method 100) of the substrate means 3, thus it doesn't necessarily define the total length of the substrate means 3 as it may in e.g. a continuous embodiment extend even longer than the length L1. It should be noted that the term "dewatering pressure" may be interchanged with the tem "suction".

Further referring to the apparatus in Figure 2 performing the method 100. The first vacuum unit 9 may be configured to apply a first dewatering pressure, wherein the second vacuum unit 9' is configured to apply a second dewatering pressure, wherein the first dewatering pressure is greater than the second dewatering pressure. The mentioned procedure allows the layer of foamed fiber furnish 2 to be treated in a continuous manner while traveling in the first direction x1. Thus, the method 100 may be performed in a continuous process. The continuous process may be performed in a manner that allows the reservoir 8 to collect liquid from the applied foamed fiber furnish 2 while traveling towards the first vacuum unit 9 where a first dewatering pressure is applied, followed by that the foamed fiber furnish continues to travel towards the second vacuum unit 9' where a second dewatering pressure is applied. The substrate means 3 may in other words travel according to a closed loop i.e., similar to how a conveyor belt operates.

Figure 6 shows the method 100 performed by the apparatus shown in Figure 3, wherein the method 100 further comprises the step of, preceding the step of applying at least one of the first and the second dewatering pressure 103, applying 105 an ultrasonic radiation to the first side of said substrate means. The ultrasonic radiation may in some embodiments be applied simultaneously as the first and/or the second vacuum unit 9, 9' are operating. Thus, the method 100 in Figure 6 comprises the steps of feeding 101 a foamed fiber furnish 2 to an apparatus 1, the apparatus 1, dispensing 102, a layer 2 of foamed fiber furnish to the first side 4 of said liquid-permeable substrate means 3, applying 105 an ultrasonic radiation to the substrate means 3, applying 103 at least a first dewatering pressure. The reservoir 8 may simultaneously intermediate/during the steps 102-105 collect 104 fluid discharge for a first period of time based on at least the thickness of the layer 2.

The configuration of fibers in the bulk of the structure can be described by fiber orientation distribution of all fibers using a pair of angles (θ, Φ), shown in exemplary Figures 7A-7B, where 7A illustrates a representation of a single fiber orientation in a 2D structure and 7B illustrates a single fiber orientation in a 3D fibrous structure (which is obtained by the method of the present disclosure). For every fiber denoted i, θ*ᵢ* is the angle between Z-axis and the fiber, and Φ*ᵢ* is the angle between X-axis and the projection of the fiber on the XY-plane (disclosed in Fig. 7A-7B). The angle Φ may have any random value in both 2D and 3D structures, however, in 2D structure θ ≅ 90°.

## Claims

1. A method (100) for producing 3D fiber structures, the method (100) comprising:
- feeding (101) a foamed fiber furnish (2) to an apparatus (1), the apparatus (1) comprising:
- a liquid-permeable substrate means (3) having a first side (4) and an opposing second side (5);
- a dispenser (6) having an outlet (7), wherein at least one of the dispenser (6) and the substrate means (3) travel with respect to the other;
- dispensing (102), by means of the dispenser (6), a layer (2) of foamed fiber furnish to the first side of said liquid-permeable substrate means (3), so to obtain a fibrous mat, wherein the apparatus (1) further comprises at least a reservoir (8) and a first vacuum unit (9) associated with the second side (5) of the liquid-permeable substrate means (3) so to collect fluid discharge from the dispensed layer (2) of fibrous mat;
- applying (103) at least a first dewatering pressure to at least a part of the second side (5) of said substrate means (3);
wherein the layer (2) of fibrous mat is dispensed so to comprise a predefined substantially uniform thickness, wherein the apparatus (1) is configured to, preceding the step of applying (103) the first dewatering pressure:
- by means of the reservoir, collect (104) fluid discharge for a first period of time based on at least the thickness of the layer (2);
wherein the first dewatering pressure is applied for a second period of time, wherein the first dewatering pressure is within the range of 70 kPa - 100 kPa,
wherein the first period of time is 1-10 minutes, wherein the second period of time is 2-10 minutes, wherein the thickness of the layer is within the range of 1-10 cm.

2. The method (100) according to claim 1, wherein the liquid-permeable substrate means travels in a first direction along a length (L1) defined by at least a first and a second portion (15', 15"), wherein the dispenser (6) is arranged to be above the first side of the substrate means (3) in said first portion (15'), wherein the reservoir (8) is arranged in said first portion (15'), wherein the first vacuum unit (9) and a second vacuum unit (9') are arranged sequentially along the length (L1) in said second portion (15"), wherein the first vacuum unit (9) is closer to the reservoir (8) than the second vacuum unit (9').

3. The method (100) according to claim 2, wherein the first vacuum unit (9) is configured to apply the e first dewatering pressure, wherein the second vacuum unit (9') is configured to apply a second dewatering pressure, wherein the first dewatering pressure is greater than the second dewatering pressure.

4. The method (100) according to claim 3, wherein the second dewatering pressure is within a range of 50 kPa - 80 kPa.

5. The method (100) according to any of the claims 1-4, wherein the method (100) further comprises the step of, preceding the step of applying the first dewatering pressure (103):
- applying (105) an ultrasonic radiation towards the substrate means (3).

6. The method (100) according to any one of the claims 2-5, wherein the method (100) is performed in a continuous process.

7. The method (100) according to any one of the preceding claims, wherein the foamed fiber furnish comprises a fiber consistency in the range of 0.5-10% based on a dry weight of the fibers, wherein the foamed fiber furnish comprises a total concentration of foaming agents in the range of 0.05-2 g/l, wherein the foamed fiber furnish comprises an air content in the range of 55-70% by volume, wherein the foamed fiber furnish is generated from a pulp slurry.

## Patentansprüche

1. Verfahren (100) zum Herstellen von 3D-Faserstrukturen, wobei das Verfahren (100) umfasst:
- Zuführen (101) eines geschäumten Faserstoffs (2) zu einer Einrichtung (1), wobei die Einrichtung (1) umfasst:
- ein flüssigkeitsdurchlässiges Substratmittel (3) mit einer ersten Seite (4) und einer gegenüberliegenden zweiten Seite (5);
- eine Ausgabeeinheit (6) mit einem Auslass (7), wobei sich mindestens eines der Ausgabeeinheit (6) und des Substratmittels (3) relativ zu dem anderen bewegt;
- Ausgeben (102) einer Schicht (2) aus geschäumtem Faserstoff, mittels der Ausgabeeinheit (6) auf die erste Seite des flüssigkeitsdurchlässigen Substratmittels (3), um eine Fasermatte zu erhalten, wobei die Einrichtung (1) ferner mindestens ein Reservoir (8) und eine erste Vakuumeinheit (9) umfasst, die der zweiten Seite (5) des flüssigkeitsdurchlässigen Substratmittels (3) zugeordnet ist, um Flüssigkeitsaustrag aus der ausgegebenen Schicht (2) der Fasermatte zu sammeln;
- Aufbringen (103) mindestens eines ersten Entwässerungsdrucks auf zumindest einen Teil der zweiten Seite (5) des Substratmittels (3);
wobei die Schicht (2) der Fasermatte so dosiert wird, dass sie eine vorgegebene im Wesentlichen gleichmäßige Dicke aufweist, wobei die Einrichtung (1) dazu ausgelegt ist, vor dem Schritt des Aufbringens (103) des ersten Entwässerungsdrucks:
- Sammeln (104) eines Fluidaustrags für eine erste Zeitdauer mittels des Reservoirs basierend auf zumindest der Dicke der Schicht (2);
wobei der erste Entwässerungsdruck für eine zweite Zeitdauer aufgebracht wird, wobei der erste Entwässerungsdruck im Bereich von 70 kPa bis 100 kPa liegt, wobei die erste Zeitdauer 1 bis 10 Minuten beträgt, wobei die zweite Zeitdauer 2 bis 10 Minuten beträgt, wobei die Dicke der Schicht im Bereich von 1 bis 10 cm liegt.

2. Verfahren (100) nach Anspruch 1, wobei sich das flüssigkeitsdurchlässige Substratmittel in einer ersten Richtung entlang einer Länge (L1) bewegt, die durch zumindest einen ersten und einen zweiten Abschnitt (15', 15") definiert ist, wobei die Ausgabeeinheit (6) so angeordnet ist, dass sie sich über der ersten Seite des Substratmittels (3) in dem ersten Abschnitt (15') befindet, wobei das Reservoir (8) in dem ersten Abschnitt (15') angeordnet ist, wobei die erste Vakuumeinheit (9) und eine zweite Vakuumeinheit (9') entlang der Länge (L1) in dem zweiten Abschnitt (15") hintereinander angeordnet sind, wobei die erste Vakuumeinheit (9) näher an dem Reservoir (8) als die zweite Vakuumeinheit (9') liegt.

3. Verfahren (100) nach Anspruch 2, wobei die erste Vakuumeinheit (9) dazu ausgelegt ist, den ersten Entwässerungsdruck
aufzubringen, wobei die zweite Vakuumeinheit
(9') dazu ausgelegt ist, einen zweiten Entwässerungsdruck aufzubringen, wobei der erste Entwässerungsdruck größer als der zweite Entwässerungsdruck ist.

4. Verfahren (100) nach Anspruch 3, wobei der zweite Entwässerungsdruck in einem Bereich von 50 kPa bis 80 kPa liegt.

5. Verfahren (100) nach einem der Ansprüche 1 bis 4, wobei das Verfahren (100) vor dem Schritt des Aufbringens des ersten Entwässerungsdrucks (103) ferner den Schritt umfasst:
- Aufbringen (105) einer Ultraschallstrahlung auf das Substratmittel (3).

6. Verfahren (100) nach einem der Ansprüche 2 bis 5, wobei das Verfahren (100) in einem kontinuierlichen Prozess durchgeführt wird.

7. Verfahren (100) nach einem der vorhergehenden Ansprüche, wobei der geschäumte Faserstoff eine Faserkonsistenz im Bereich von 0,5 bis 10 % bezogen auf das Trockengewicht der Fasern umfasst, wobei der geschäumte Faserstoff eine Gesamtkonzentration von Schaummitteln im Bereich von 0,05 bis 2 g/l umfasst, wobei der geschäumte Faserstoff einen Luftgehalt im Bereich von 55 bis 70 Vol.-% umfasst, wobei der geschäumte Faserstoff aus einer Zellstoffsuspension erzeugt wird.

## Revendications

1. Procédé (100) de production de structures de fibres 3D, le procédé (100) comprenant :
- l'alimentation (101) d'une composition de fibres moussée (2) vers un appareil (1), l'appareil (1) comprenant :
- un moyen formant substrat perméable aux liquides (3) présentant un premier côté (4) et un second côté opposé (5) ;
- un distributeur (6) ayant une sortie (7), dans lequel au moins l'un parmi le distributeur (6) et le moyen formant substrat (3) se déplace par rapport à l'autre ;
- la distribution (102), au moyen du distributeur (6), d'une couche (2) de composition de fibres moussée sur le premier côté dudit moyen formant substrat perméable aux liquides (3), de manière à obtenir un mat fibreux, dans lequel l'appareil (1) comprend en outre au moins un réservoir (8) et une première unité de vide (9) associée au second côté (5) du moyen formant substrat perméable aux liquides (3) de manière à collecter une décharge de fluide provenant de la couche distribuée (2) de mat fibreux ;
- l'application (103) d'au moins une première pression de déshydratation sur au moins une partie du second côté (5) dudit moyen formant substrat (3) ;
dans lequel la couche (2) de mat fibreux est distribuée de manière à présenter une épaisseur prédéfinie sensiblement uniforme, dans lequel l'appareil (1) est configuré pour, avant l'étape d'application (103) de la première pression de déshydratation :
- au moyen du réservoir, collecter (104) la décharge de fluide pendant une première période de temps basée sur au moins l'épaisseur de la couche (2) ;
dans lequel la première pression de déshydratation est appliquée pendant une seconde période de temps, dans lequel la première pression de déshydratation est comprise dans la plage de 70 kPa à 100 kPa,
dans lequel la première période de temps est de 1 à 10 minutes, dans lequel la seconde période de temps est de 2 à 10 minutes, dans lequel l'épaisseur de la couche est comprise dans la plage de 1 à 10 cm.

2. Procédé (100) selon la revendication 1, dans lequel le moyen formant substrat perméable aux liquides se déplace dans une première direction le long d'une longueur (L1) définie par au moins une première et une seconde partie (15', 15"), dans lequel le distributeur (6) est agencé pour être au-dessus du premier côté du moyen formant substrat (3) dans ladite première partie (15'), dans lequel le réservoir (8) est agencé dans ladite première partie (15'), dans lequel la première unité de vide (9) et une seconde unité de vide (9') sont agencées séquentiellement le long de la longueur (L1) dans ladite seconde partie (15"), dans lequel la première unité de vide (9) est plus proche du réservoir (8) que la seconde unité de vide (9').

3. Procédé (100) selon la revendication 2, dans lequel la première unité de vide (9) est configurée pour appliquer la première pression de déshydratation, dans lequel la seconde unité de vide (9') est configurée pour appliquer une seconde pression de déshydratation, dans lequel la première pression de déshydratation est supérieure à la seconde pression de déshydratation.

4. Procédé (100) selon la revendication 3, dans lequel la seconde pression de déshydratation est comprise dans une plage de 50 kPa à 80 kPa.

5. Procédé (100) selon l'une quelconque des revendications 1 à 4, dans lequel le procédé (100) comprend en outre l'étape consistant à, avant l'étape d'application de la première pression de déshydratation (103) :
- appliquer (105) un rayonnement ultrasonore vers le moyen formant substrat (3).

6. Procédé (100) selon l'une quelconque des revendications 2 à 5, dans lequel le procédé (100) est réalisé selon un processus continu.

7. Procédé (100) selon l'une quelconque des revendications précédentes, dans lequel la composition de fibres moussée comprend une consistance de fibres dans la plage de 0,5 à 10 % sur la base d'un poids sec des fibres, dans lequel la composition de fibres moussée comprend une concentration totale d'agents moussants dans la plage de 0,05 à 2 g/l, dans lequel la composition de fibres moussée comprend une teneur en air dans la plage de 55 à 70 % en volume, dans lequel la composition de fibres moussée est générée à partir d'une suspension de pâte.
